

E. OESER,  
BRONZE FOIL,  
APPLICATION FILED MAY 1, 1911.

1,037,515.

Patented Sept. 3, 1912.

Fig. 1.



Fig. 2.



Fig. 3.



Witnesses:  
J. M. Wyntkoop.  
Ida T. Stanley.

Inventor:  
Ernst Oeser.  
By Knight  
attor

# UNITED STATES PATENT OFFICE.

ERNST OESSER, OF BERLIN, GERMANY.

## BRONZE FOIL.

1,037,515.

Specification of Letters Patent. Patented Sept. 3, 1912.

Application filed May 1, 1911. Serial No. 624,385.

To all whom it may concern:

Be it known that I, ERNST OESSER, manufacturer, a subject of the German Emperor, and resident of No. 20 Culmstrasse, Berlin, Germany, have invented certain new and useful Improvements in Bronze Foils, of which the following is a specification.

Bronze foils as they are frequently used as a substitute for leaf gold, are generally made by either applying a coat of paint consisting of a paint powder and a cement to a smooth surface say a glass plate and before such coat of paint has dried strewing bronze powder on the same, or by applying a coat of varnish to the glass plate, strewing bronze powder on said coat of varnish and again covering the said bronzed coat with varnish after any excess of bronze powder has been removed. As a varnish for the latter method generally the socalled zapon varnish or collodium is used. The bronze foil obtained by the former method, has the advantage, that it will not let the color of the object covered with it shine through; it has the disadvantage, of not being weatherproof and therefore being readily oxidized and losing its fine appearance. This is particularly the case, when the foil is employed for covering say wood, leather and other materials, which are frequently used in the open air and are therefore subject to the influences of the atmosphere. Far better results are obtained with the foil made after the second named method, particularly if the layer of bronze is subsequently covered with a coat of varnish. This latter kind of foil has, however, the disadvantage, that the color of the article covered with it, will easily shine through, so that the fiery gloss of the bronze foil is impaired. If such a foil is to be applied to the respective article by pressure and with a heated die, the foil after the latter method, not having a colored backing, will not be serviceable, as the coat of varnish consisting of collodium or zapon varnish will not suffice to securely fix the foil to the article covered with it, whereas the foil made after the former method and having a colored backing will better adhere to the article being covered with it.

The object of the present invention is to combine the advantages of the kinds of bronze foils hitherto known, and avoid their disadvantages.

The present invention consists in that the bronze foil is made according to diagram Fig-

ure 1 of three superimposed layers, namely, at the bottom a layer of coloring matter *a*, on this a layer of bronze *b* and on this a coat of varnish *c*, or according to the diagram 60 Fig. 2 of four superimposed layers, namely a coat of resin *d*, a layer of coloring matter *a*, a layer of bronze *b*, a coat of varnish *c*, or according to diagram Fig. 3 of a coat of resin *d*, a coat of varnish *c*, a layer of 65 bronze *b*, a coat of varnish *c*. In all instances the layer of coloring matter or resin is turned toward the article to be covered, the coat of varnish toward the observer. The layer of coloring matter consists of a 70 binding medium soluble in water, alcohol or ether, such as glue, dextrin, gelatin, albumen and the like, or shellac, mastic, and the like, or collodium, and of a powdered colored material (paint) mixed with this 75 binding medium, which for the purpose of affording a good covering property is preferably chosen of a white or yellowish color. After the coloring matter mixed with the binding medium has been ground so finely, 80 that it becomes applicable as a paint, it is applied by means of a brush to a well cleaned glass plate or the glass plate may be also dipped into the paint. When the coat of paint has dried so far, that it is still 85 somewhat adhesive, the bronze powder is strewn on it in known manner, the excess of bronze is brushed off, and finally a coat of varnish is applied. This coat of varnish may consist of thin liquid collodium or of 90 zapon or any other suitable material. The term zapon applies to a product in the market which is composed of celluloid tailings and a mixture of ether, alcohol and amyl-acetate. The composition of the coat of 95 varnish shall, however be considered as immaterial to the principle of the invention.

If for the purpose of obtaining a better adhesiveness of the foil, a coat or layer of resin is employed beneath the layer of coloring matter or the bottom coat of varnish, this coat of resin will preferably consist of shellac dissolved in alcohol, to which solution, if so desirable, some mastic may be added. By all means a layer of coloring matter or a coat of varnish must be interposed between this coat of resin and the layer of bronze as the resin which is fused on the foil being embossed with a hot die to the rough surface of the article under treatment would penetrate the layer of bronze and impair the fiery gloss of the same. If

the bronze foil is backed with a coat of resin, the coloring matter may in some cases be dispensed with, as it is the case with the third form according to diagram Fig. 3, 5 because the resin will have a covering power of its own, particularly if mixed with some mastic and of a yellowish or orange color.

When the bronze foil has been made in the hereinbefore described manner by subsequent application of the several layers and coats and after all these have dried completely, the whole is detached by means of a spattle, a painter's tool resembling a plane iron, from the glass plate. The thus detached bronze foil is spread the same as a piece of leaf gold between two sheets of paper and kept there until it is to be used.

The foil is used by laying it on the object to be covered and pressing it to the same by means of a suitably engraved and if necessary heated die. After pressing the parts of foil projecting beyond the embossed pattern are removed with a soft brush. If,

however, the foil is to be used for covering a wall, a stone or a large piece of metal, a suitable cementing medium will have to be previously applied to the respective article, the same as with leaf gold, whereupon the foil is applied and any excess is removed after this cementing medium has dried. 39

I claim:

A bronze foil protected against oxidization as a substitute for leaf metal, consisting of a foundation of coloring matter and a binding material as a backing, a layer of bronze on said coloring matter, a resinous covering beneath the backing of the coloring matter and a coat of varnish on said bronze. 35

The foregoing specification signed at Berlin, Germany, this nineteenth day of April, 1911.

ERNST OESER.

In presence of—

HENRY HASPER,  
WOLDEMAR HAUPT.